# EUROPEAN PATENT APPLICATION

(11) **EP 0 479 487 A1**
(43) Date of publication of application: **08.04.1992**
(21) Application number: 91308768.0
(22) Date of filing: 26.09.1991
(51) Int. Cl.: C10L 5/10

(54) **Briquettes**

(30) Priority: 27.09.1990 ZA 907741; 30.04.1991 ZA 913288
(71) Applicant: Botha, Gary, Roodepoort, Transvaal Province (ZA); Nesbitt, Dennis Bertram, Sandton, Transvaal Province (ZA)
(72) Inventor: Botha, Gary, Roodepoort, Transvaal Province (ZA); Nesbitt, Dennis Bertram, Sandton, Transvaal Province (ZA)
(74) Representative: Gaunt, Robert John

(57) **Abstract**

A briquette comprises, in admixture with one another and as a unitary mass, a particulate carbonaceous material, a binder, and at least one sodium compound capable of inhibiting disintegration of the unitary mass at high temperature at least for a period of time. The sodium compound is not sodium nitrate or sodium silicate.

## Description

THIS INVENTION relates to briquettes. It relates also to a method of making briquettes.

According to a first aspect of the invention, there is provided a briquette which comprises, in admixture with one another and as a unitary mass, a particulate carbonaceous material, a binder, and at least one sodium compound capable of inhibiting disintegration of the unitary mass at high temperature at least for a period of time, with the proviso that the sodium compound is not sodium nitrate or sodium silicate.

The carbonaceous material may comprise bituminous coal, anthracite, coke, char, charcoal, or the like. The particles of carbonaceous material may be less than 6 mm in size, preferably less than 3 mm in size, ie capable of passing through 3 mm diameter screen or mesh openings. In use, the carbonaceous material acts as solid fuel and as a reductant, eg when the briquette is used in iron or steel smelting.

The binder may be starch based, and may also be in particulate form initially. The starch based binder may initially be in modified or unmodified form. If it is initially in unmodified form, it may be pretreated prior to use, by heating it, thereby to render it into modified form. The binder particles may initially be less than 1 mm, eg about 0.5 to 0.8 mm in size. The unitary mass can then be obtained by heating the admixture of the constituents sufficiently to form a compressible mix, and compressing the mix into the unitary mass.

The sodium compound may be sodium hydroxide, which may initially be in solid or liquid form. The sodium hydroxide is thus believed to act as a stabilizing agent for inhibiting disintegration of the briquettes at high burning temperatures, at least for a period of time.

The briquette may also include sodium nitrate in admixture with the carbonaceous material, binder and sodium hydroxide. The sodium nitrate is believed to control the rate of burning of the briquette so that it lasts longer.

The briquette may comprise, on a mass basis
- carbonaceous material: - 80-95%
- binder: - 5-15%
- sodium hydroxide: - 0.05-5%
- sodium nitrate: - 0.1-10%

The briquette may include a waterproofing agent in admixture with the other constituents. When present, the waterproofing agent may be present in a proportion of 1-50%, based on the binder.

The waterproofing agent may be colloidal silica, for example an aqueous colloidal dispersion of silica particles available as several grades in South Africa under the name "LUDOX" (registered trade mark) from Chempro (Proprietary) Limited (ex. Du Pont Co.). Suitable grades are "LUDOX HS-30", "LUDOX HS-40" and "LUDOX SM".

The briquette may also include, instead of the waterproofing agent or in addition thereto, fines in admixture with the other constituents. When present, the fines may be present in a proportion of 20-75% by mass.

The fines may comprise particles of chromite, magnesia, dolomite, limestone, ferro-silicon, flux, manganese, silicon metal, pure silica, quartz, or the like, or mixtures thereof. The fines particles may be less than 6 mm in size, preferably less than 3 mm in size.

When the briquette contains the waterproofing agent and the fines, it may comprise, on a mass basis
- carbonaceous material: - 20-70%
- fines: - 20-75%
- binder: - 5-15%
- waterproofing agent: - 1-50%
(based on binder)
- sodium hydroxide: - 0.05-5%

According to a second aspect of the invention, there is provided a briquette which comprises, in admixture with one another and as a unitary mass, a particulate carbonaceous material, a binder, a waterproofing agent, and at least one sodium compound capable of inhibiting disintegration of the unitary mass at high temperatures at least for a period of time, with the proviso that the sodium compound is not sodium nitrate or sodium silicate.

The carbonaceous material, binder, waterproofing agent and sodium compound may be as hereinbefore described, and the briquette may also include fines as hereinbefore described.

According to a third aspect of the invention, there is provided a briquette which comprises, in admixture with one another and as a unitary mass, a particulate carbonaceous material, fines, a binder, and at least one sodium compound capable of inhibiting disintegration of the unitary mass at high temperatures at least for a period of time, with the proviso that the sodium compound is not sodium nitrate or sodium silicate.

The carbonaceous material, binder, fines and sodium compound may be as hereinbefore described.

According to a fourth aspect of the invention, there is provided a briquette which comprises, in admixture with one another and as a unitary mass, a particulate carbonaceous material, fines, a binder, a waterproofing agent, and at least one sodium compound capable of inhibiting disintegration of the unitary mass at high temperatures at least for a period of time, with the proviso that the sodium compound is not sodium nitrate or sodium silicate.

The carbonaceous material, fines, binder, waterproofing agent and sodium compound may be as hereinbefore described.

According to a fifth aspect of the invention, there is provided a method of making a briquette, which comprises
admixing a particulate carbonaceous material, a binder, and at least one sodium compound capable of inhibiting disintegration of the briquette at high temperatures at least for a period of time, with the proviso that the sodium compound is not sodium nitrate or sodium silicate;
heating the admixture sufficiently to form a compressible mix;
compressing the mix into a green briquette;
curing the green briquette.

The admixture may comprise particulate carbonaceous material, a binder, sodium hydroxide and sodium nitrate. A premix can be formed by admixing the binder, sodium hydroxide and sodium nitrate. Thereafter this premix can be admixed with the particulate carbonaceous material.

The resultant mixture may be heated to at least 50°C, eg to between 50°C and 100°C, typically in the range of 70-72°C. The heating may be direct steam heating, so that the mixture is thereby moistened at least to a degree. Typically, it may then contain about 20% by mass water after the heating has been completed. The compression may be effected at a pressure of between 0.5 and 10 tonnes, and the maximum dimension of the resultant briquette may be about 2 to 20 cm.

The curing may be effected in a curing tunnel, and the curing temperature may be at least 100°C, eg between 150°C and 350°C. The curing can, however, also be effected at room temperature, if desired.

According to a sixth aspect of the invention, there is provided a method of making a briquette, which comprises
admixing a particulate carbonaceous material, fines, a binder, a waterproofing agent, and at least one sodium compound capable of inhibiting disintegration of the briquette at high temperatures at least for a period of time, with the proviso that the sodium compound is not sodium nitrate or sodium silicate;
heating the admixture sufficiently to form a compressible mix;
compressing the mix into a green briquette;
and curing the green briquette.

A first premix can be formed by admixing the particulate carbonaceous material and the fines, and a second premix can be formed by admixing the binder, the waterproofing agent and the sodium compound. Thereafter, the first premix can be admixed with the second premix.

The resultant mixture may be heated to at least 50°C, as hereinbefore described.

According to a seventh aspect of the invention, there is provided a method of making a briquette, which comprises
admixing a particulate carbonaceous material, a binder, a waterproofing agent, and at least one sodium compound capable of inhibiting disintegration of the briquette at high temperatures at least for a period of time, with the proviso that the sodium compound is not sodium nitrate or sodium silicate;
heating the admixture sufficiently to form a compressible mix;
compressing the mix into a green briquette;
and curing the green briquette.

According to an eighth aspect of the invention, there is provided a method of making a briquette, which comprises
admixing the particulate carbonaceous material, fines, a binder, and at least one sodium compound capable of inhibiting disintegration of the briquette at high temperatures at least for a period of time, with the proviso that the sodium compound is not sodium nitrate or sodium silicate;
heating the admixture sufficiently to form a compressible mix;
compressing the mix into a green briquette;
and curing the green briquette.

The invention will now be described by way of example with reference to the accompanying drawings.

In the drawings,
FIGURE 1 shows a block diagram depicting the steps in a method of forming briquettes in accordance with one embodiment of the invention; and
FIGURE 2 shows a similar block diagram depicting the steps in a method of forming briquettes in accordance with another embodiment of the invention.

Referring to Figure 1, reference numeral 10 generally indicates the steps in a method of forming briquettes in accordance with one embodiment of the invention.

In Figure 1, reference numeral 11 indicates a char preparation stage, while reference numeral 12 indicates a binder preparation stage. A transfer line 14 interconnects the stage 12 with a mixing stage 16 with sodium hydroxide and sodium nitrate feed lines 18, 20 respectively leading into the mixing stage 16. A transfer line 22 leads from the mixing stage 16 to a further mixing stage 24, with a transfer line 26 also leading from the stage 11 to the mixing stage 24.

A transfer line 28 leads from the mixing stage 24 to a heating stage 30, with a steam flow line 32 leading into the heating stage 30. A transfer or flow line 34 leads from the mixing stage 30 to a press 36, while a transfer line 38 leads from the press 36 to a curing stage 40 in the form of a curing tunnel.

In use, char is milled down in the stage 11 to a particle size less than 3 mm, ie so that its particles can pass through 3 mm diameter screen openings.

In the stage 12, sorghum grains or kernels are milled down to 0.8 mm, ie so that they pass through 0.8 mm mesh or screen openings. Instead, they can be milled down to 0.5 mm if desired. If desired, they can be de-hulled first. Furthermore, the milled sorghum binder can, if desired, first be modified by subjecting it to heat treatment, ie cooking it, if in unmodified form. However, it can also be used in unmodified form. The particulate sorghum binder passes along the transfer line 14 to the mixing stage 16, where it is admixed with sodium hydroxide and sodium nitrate particles or powder. The resultant premix passes along the transfer line 22 to the mixing stage 24 where it is admixed with the particulate solid carbonaceous material. The constituents are present in the resultant mixture in the stage 24 in the following proportions by mass:
- particulate char: - 90%
- sorghum binder: - 9.5%
- sodium hydroxide: - 0.1%
- sodium nitrate: - 0.4%

This mixture passes along the transfer line 28 to the heating stage 30 where it is heated by direct steam heating, with the steam heat entering along the flow line 32. The mixture is heated to 70-72°C, and as a result of the direct steam heating then has a moisture content of about 20%.

The moist mix passes along the transfer line 34 to the press 36, where it is pressed into briquettes having a maximum dimension of about 2 to 20 cm, at a pressure of 0.5 to 10 tonnes, depending on the size of the briquettes, to form green briquettes. The green briquettes pass along the transfer line 38 to the curing tunnel 40 which is provided with suitable heating means (not shown) for heating the briquettes to 150°C, thereby to cure them.

To the briquette mix can be added from 1-50% by mass (based on binder) LUDOX HS-30 as waterproofing agent and/or from 20-75% by mass fines.

The Applicants believe that these briquettes will find particular application in reduction processes such as iron and steel making, where the char will also act as a reductant. The sodium hydroxide acts in stabilizing the briquettes so that they do not readily disintegrate at the high temperatures required in iron and steel reduction processes at least for an initial period of time. The sodium nitrate acts in ensuring a better distribution of heat within the briquettes, thereby controlling the rate of burning of the briquettes and ensuring that they have a longer life.

The briquettes can also be used for domestic purposes.

Referring to Figure 2, reference numeral 100 generally indicates the steps in a method of forming briquettes in accordance with another embodiment of the invention.

Parts of Figure 2 which are the same or similar to those of Figure 1 are indicated with the same reference numerals.

In Figure 2, reference numeral 11 again indicates a coke preparation and mixing stage, with a fines feed line 102 leading into it. Reference numeral 12 again indicates a binder preparation and mixing stage, with a colloidal silica feed line 104 leading into it. As in Figure 1, a transfer line 14 interconnects the stage 12 with a mixing stage 16, with a sodium hydroxide feed line 18 leading into the mixing stage 16. A transfer line 22 leads from the mixing stage 16 to a further mixing stage 24, with a transfer line 26 also leading from the stage 11 to the mixing stage 24; a transfer line 28 leads from the mixing stage 24 to a heating stage 30, with a steam flow line 32 leading into the heating stage 30; a transfer or flow line 34 leads from the mixing stage 30 to a press 36, while a transfer line 38 leads from the press 36 to a curing stage 40 in the form of a curing tunnel.

In use, coke is milled down in the stage 11 to have a particle size less than 3 mm, and admixed with fines to form a first premix.

In the stage 12, sorghum grains or kernels are milled down to 0.5 mm, and admixed with "LUDOX HS-30" (registered trade mark), which is an aqueous colloidal dispersion of silica particles available in South Africa from Chempro (Proprietary) Limited (ex. Du Pont Co.). If desired, the sorghum grains or kernels can be de-hulled first. The binder / "LUDOX HS-30" mix passes along the transfer line 14 to the mixing stage 16, where it is admixed with sodium hydroxide particles or powder. The resultant second premix passes along the transfer line 22 to the mixing stage 24 where it is admixed with the first premix. The constituents are present in the resultant mixture in the stage 24 in the following proportions, by mass:
- particulate coke breeze: - 30
- chromite fines: - 100
- limestone fines: - 10
- quartz fines: - 3
- sorghum binder: - 9.5
- "LUDOX HS-30": - 2.0
- sodium hydroxide: - 0.1

This mixture passes along the transfer line 28 to the heating stage 30 where it is heated by direct steam heating, with the steam heat entering along the flow line 32. The mixture is heated to 70-72°C, and as a result of the direct steam heating then has a moisture content of about 20%.

The moist mix passes along the transfer line 34 to the press 36, where it is pressed into briquettes having a maximum dimension of about 2 to 20 cm, at a pressure of 0.5 to 10 tonnes, depending on the size of the briquettes, to form green briquettes. The green briquettes pass along the transfer line 38 to the curing tunnel 40 which is provided with suitable heating means (not shown) for heating the briquettes to 150°C, thereby to cure them.

The above Example was repeated successfully, firstly replacing the chromite fines only by magnesia fines, and secondly replacing both the chromite fines and the limestone fines by ferrosilicon fines. In the above example, the limestone fines and quartz fines can be omitted if desired. Instead or additionally, the LUDOX HS-30 can be omitted if desired. Still further, all the fines can be omitted for particular applications.

Tests conducted on the briquettes showed that when they were immersed in water for 1 and 2 weeks, the briquettes still maintained their integrity.

As mentioned hereinbefore, the Applicants believe that the briquettes according to the invention will find particular application in iron and steel making, where the product can act as a composite feed to a submerged arc furnace. The fines are readily available in South Africa as a waste product thereby reducing the manufacturing costs of the briquettes as well as reduction process processing costs when the briquettes are used in reduction processes. The briquettes also provide an effective manner of introducing additives required for the reduction process, eg chrome required to be added to iron in steelmaking, to the furnace. Further, the use of colloidal silica provides briquettes with sufficient waterproofing properties to permit the briquettes to be stored outside.

Furthermore, the Applicants have found that by using the combination of starch as binder and sodium hydroxide, as hereinbefore described, very stable briquettes which did not disintegrate at temperatures of about 2000°C were obtained. In contrast, similar briquettes having a combination of starch, molasses and clay (bentonite) as binder, disintegrated at about 600°C. Still further, both starch and sodium hydroxide provide very little residue at elevated temperatures leading to a very pure final product or briquette, in contrast to briquettes derived from molasses and/or clay which have high proportions of impurities such as ash, sulphur and phosphorus.

## Claims

1. A briquette characterized in that it comprises, in admixture with one another and as a unitary mass, a particulate carbonaceous material, a binder, and at least one sodium compound capable of inhibiting disintegration of the unitary mass at high temperature at least for a period of time, with the proviso that the sodium compound is not sodium nitrate or sodium silicate.

2. A briquette in accordance with Claim 1, characterized in that the carbonaceous material comprises bituminous coal, anthracite, coke, char or charcoal, with the particles being less than 6 mm in size, with the binder being starch based and the sodium compound being sodium hydroxide.

3. A briquette in accordance with Claim 2, characterized in that it comprises, on a mass basis
carbonaceous material - 80-95%
binder - 5-15%
sodium hydroxide - 0.05-5%
sodium nitrate - 0.1-10%

4. A briquette in accordance with Claim 2, characterized in that it includes a waterproofing agent in admixture with the carbonaceous material, the binder, and the sodium compound.

5. A briquette in accordance with Claim 4, characterized in that it includes fines in admixture with the carbonaceous material, binder, sodium compound and waterproofing agent, with the briquette comprising, on a mass basis,
carbonaceous material - 20-70%
fines - 20-75%
binder - 5-15%
waterproofing agent - 1-50%
(based on binder)
sodium hydroxide - 0.05-5%

6. A briquette in accordance with Claim 2, characterized in that it includes fines in admixture with the carbonaceous material, binder, and the sodium compound.

7. A briquette in accordance with Claim 5 or Claim 6, characterized in that the fines comprise particles of chromite, magnesia, dolomite, limestone, ferro-silicon, flux, manganese, silicon metal, pure silica, quartz, or mixtures thereof, with the particles being less than 6 mm in size.

8. A briquette characterized in that it comprises, in admixture with one another and as a unitary mass, a particulate carbonaceous material; a binder; a waterproofing agent and/or fines; and at least one sodium compound capable of inhibiting disintegration of the unitary mass at high temperatures at least for a period of time, with the proviso that the sodium compound is not sodium nitrate or sodium silicate.

9. A method of making a briquette, characterized in that it comprises
admixing a particulate carbonaceous material, a binder, and at least one sodium compound capable of inhibiting disintegration of the briquette at high temperatures at least for a period of time, with the proviso that the sodium compound is not sodium nitrate;
heating the admixture sufficiently to form a compressible mix;
compressing the mix into a green briquette;
curing the green briquette.

10. A method according to Claim 9, characterized in that the mixture is heated to at least 50°C by direct steam heating, with the curing being effected in a curing tunnel at a temperature of at least 100°C.
